

## UNITED STATES PATENT OFFICE.

MARIA SCHOLZ, OF LEICHLINGEN, GERMANY.

## BATIK ART.

No Drawing.

Application filed June 25, 1923. Serial No. 647,760.

*To all whom it may concern:*

Be it known that I, MARIA SCHOLZ, a citizen of Germany, residing at Leichlingen, Rhenish Prussia, Germany, have invented 5 certain new and useful Improvements in the Batik Art, for which I have filed an application for patent in Germany, June 29, 1922, and of which the following is a specification.

In the batik art, as well known, the 10 tile fabric is first provided with a wax pattern and is then dyed, the waxed portions, which do not absorb the dyestuff, retaining their original color tone. The wax is subsequently suitably removed. Further, in 15 cloth-printing it is known to print upon the dyed fabric a pattern by means of a discharge medium, the latter by bleaching the ground color at the places so imprinted then producing the pattern.

20 These decolored prints, which have become very popular in the cloth-printing industry, have so far not been found usable to any extent in the batik art for the main reason that the fabric imprinted with the discharge pattern must finally be treated in a 25 steam chamber or the Mather-Platt apparatus to fix the colors. If goods pattern partly with discharge and partly with wax would be thus steamed the wax, obviously, 30 would melt and spread over the discharged portions since the discharges, as usually compounded for the imprinting process, do not possess sufficient wax repelling power to prevent this, with the result that the 35 goods subsequently could not properly be dyed, or the wax would run off so quickly that the discharge would have no time to destroy the dyestuff.

40 The present invention is based principally on the discovery that the discharges employed in the cloth-printing art, especially the hydrosulphites, such as for instance the formaldehydsulfoxylat



45 which is known as rongalit, which are employable for most all dischargeable dyes and for all fabrics, can be very well utilized in the batik art. It has been found 50 that when the discharge-patterned material is passed through a wax bath heated to about 80 degrees centigrade, the dyestuff is readily and effectively destroyed at the discharged places, the destruction of the dye 55 being not only complete but also practically

instantaneous, whereas in the old steaming process at least 5 minutes were required to bring this about.

I will now describe in detail the several steps entering into the new process so that 60 anyone skilled in the art, by proceeding according to this description, will have the best results and turn out high-grade work of the character set forth.

If, for instance, a red pattern is desired 65 on a green ground, the entire piece of fabric is first dyed green in well known manner, whereupon the pattern is imprinted upon it with a suitable discharge, as well known in the art, on the printing machine, 70 by hand, or by stenciling or otherwise. For reasons further below given it is necessary to add to the discharge a wax repellent, such as for instance tragacanth thickening, which has been found eminently suitable. 75

When employing the above specified rongalit as discharge medium the following combination will be found suitable: 100 grams rongalit, 350 grams gum, 100 grams water, 500 grams tragacanth thickening, 80 comprising a solution of about 65 parts tragacanth in 1000 parts water.

This formula is given merely by way of example, having been found eminently suitable for the purpose, and, obviously, variations in the composition may be made within limits; for instance I may omit the admixture of the gum in certain instances. 85

The discharge-patterned fabric is then passed through a hot wax bath in which 90 the ground is waxed, whereupon the fabric is placed into a cold water bath, wherein the waxed portions will set and the wax-free discharged portions are thoroughly rinsed and thus freed of the discharge. Next, the 95 fabric is manipulated in the manner well known in the batik art, to produce fine cracks and fissures in the cold wax layer. The fabric is then passed into the second dye bath, which in our case would be red, 100 wherein the discharged and thus wax-free portions representing the pattern are dyed and then show the pattern in red, whilst at the same time the dye penetrates through the breaks and fissures and produces on the 105 waxed fabric portions the vein or marble effect so highly valued in the batik art.

The discharged portions will show the pattern in the pure red tone, but the veining will show a compound coloring of the red 110

of the pattern and the green of the ground. The dyeing process being completed, the wax is removed from the fabric in suitable manner, for instance by hot-ironing or dissolving-out. The finished product shows a red pattern on a green base with the latter showing veins of the combination of the two colors. In order that the discharged portions are thoroughly permeated by the dye 10 of the second bath, care must be taken to keep these fabric portions devoid of wax. This can best be obtained by adding to the discharge a tragacanth thickening or a similar wax repelling medium.

15 If it is desired to produce an additional pattern, and this also on the wax-free discharged pattern, the fabric, after having left the second color (red) bath, can again be passed through a second wax bath where- 20 in the entire fabric is impregnated and covered with the wax. If now this second wax coating is hardened in cold water and the fabric then gathered to produce cracks and breaks and is then introduced into a third 25 color bath, then an additional marble effect is obtained extending over the entire fabric including the previously discharged portions and showing a compound color effect depending upon the color tone of the ground 30 at these portions.

A further patterning may be obtained by imprinting, beside the discharge pattern, a second pattern with a wax repellent, for instance a tragacanth thickening, but without 35 discharge admixture. The pattern thus produced will show the combination coloring of the ground with the second dye bath color, that is to say, the same tint as the veins showing on the colored ground. The 40 application of these two imprints can also be effected simultaneously in the well known multi-color printing press.

In producing discharge patterns by the imprinting machine the engraved portion 45 of the roller should preferably to sunk at least 1 millimeter deeper than usual.

The above process is of special value in the treatment of heavy fabrics, such as wool-plush, velvet and the like, since in the dye 50 bath the pattern is completely dyed-through, a result unobtainable when the patterning is produced with printing dye.

What I claim is:—

1. In the batik art, the described step 55 which comprises patterning the pre-dyed material, prior to treating it in a wax bath, with a discharge containing a wax repellent.

2. In the batik art, the described steps 60 which comprise patterning the predyed material with rongalit having an admixture of a wax repellent, and then passing the thus patterned material into a wax bath.

3. In the batik art, the described steps 65 which comprise patterning the predyed material with a discharge thickened with

tragacanth, and then passing the thus patterned material into a wax bath.

4. In the batik art, the described steps which comprise patterning the predyed material with a discharge medium containing 70 a wax repellent, passing the thus patterned material through a wax bath, suitably breaking the wax, passing the material through a dye bath, and finally dewaxing the material. 75

5. In the batik art, the described steps which comprise patterning the predyed material partly with a discharge thickened with a wax repellent, and partly with a plain wax repellent, and then passing the 80 thus patterned material through a wax bath. 85

6. In the batik art, the described steps which comprise patterning the predyed material partly with a discharge containing a wax repellent, and partly with a tragacanth thickening, and then passing the thus patterned material through a wax bath. 90

7. In the batik art, the described steps which comprise patterning the predyed material with a discharge having incorporated 95 therein a wax repellent, and then passing the thus patterned fabric into a wax bath heated to about 80° C. 100

8. In the batik art, the described steps which comprise patterning the predyed material partly with a discharge containing a wax repellent, and partly with a plain wax repellent, and then passing the thus patterned material into a wax bath heated to 105 about 80° C. 110

9. In the batik art, the described steps which comprise patterning the predyed material with a discharge composed of 1 part by weight of rongalit and 5 parts of tragacanth thickening, and then passing the thus patterned material into a wax bath. 115

10. In the batik art, the described steps which comprise patterning the predyed material with a discharge composed of 1 part by weight of rongalit, 3½ parts of gum, 1 part of water, and 5 parts tragacanth thickening, and then passing the thus patterned material into a wax bath. 120

11. In the batik art, the described steps which comprise patterning the predyed material with a discharge of 1 part by weight of rongalit, 3½ parts of gum, 1 part of water, and 5 parts of tragacanth thickening, and then passing the thus patterned material into a wax bath heated to about 80° C. 125

12. In the batik art, the described steps which comprise treating the material in a first dye bath, patterning the dyed material in part with a discharge containing a wax repellent, and in part with a plain wax repellent, passing the thus patterned material through the wax bath, breaking the wax, treating the fabric in a second dye bath, and finally dewaxing the fabric. 130

13. In the batik art, the described steps

which comprise treating the material in a first dye bath, patterning the dyed material in part with a discharge containing a wax repellent, and in part with a plain wax repellent, passing the thus patterned material through a wax bath, breaking the wax, treating the fabric in a second dye bath, dewaxing the fabric, passing the fabric through a second wax bath, again breaking the wax, treating the fabric in a third dye bath, and finally dewaxing the fabric.

In testimony whereof I affix my signature.

MARIA SCHOLZ.